

March 26, 1940.

L. W. GODDU ET AL

2,194,546

DIAMOND LAP

Filed Nov. 4, 1937

2 Sheets-Sheet 1



FIG. I



FIG. II



FIG. III

FIG. IV



FIG. V

FIG. VI



FIG. VII

INVENTOR  
WILLIAM J. WRIGHTON  
LLOYD W. GODDU  
BY

Harry H. Stell  
ATTORNEY

March 26, 1940.

L. W. GODDU ET AL

2,194,546

DIAMOND LAP

Filed Nov. 4, 1937

2 Sheets-Sheet 2



FIG. IX



FIG. X



FIG. XI



FIG. XII



FIG. XIII

INVENTOR  
WILLIAM J. WRIGHTON  
LLOYD W. GODDU  
BY

*Harry H. Styll*  
ATTORNEY

## UNITED STATES PATENT OFFICE

2,194,546

## DIAMOND LAP

Lloyd W. Goddu and William J. Wrighton,  
Southbridge, Mass., assignors to American Optical Company, Southbridge, Mass., a voluntary association of Massachusetts

Application November 4, 1937, Serial No. 172,800

3 Claims. (Cl. 51—278)

This invention relates to diamond laps and to a method for making the same.

An object of the invention is to improve the wearing qualities of the diamond laps thus produced.

In the accompanying drawings which illustrate our invention Fig. I is a perspective view of a diamond lap;

Fig. II is a plan view of sheet metal carrying the diamond particles;

Fig. III is an end view illustrating the assembly of such a sheet with a core;

Fig. IV is a diagrammatic sectional view illustrating the insertion of the diamond carrying metal into the body of the lap;

Fig. V is a plan view illustrating the impregnating of wire mesh with diamond particles;

Fig. VI is a detail sectional view on an enlarged scale illustrating the fixing of the diamond particles in the wire mesh;

Fig. VII is a diagrammatic sectional view illustrating the insertion of the diamond impregnated mesh in the lap;

Fig. VIII is a view similar to Fig. IV illustrating the insertion of a diamond carrying mixture into the lap;

Fig. IX is a plan view of wire mesh impregnated with diamond particles;

Fig. X is a plan view of a lap having a plurality of layers of diamond impregnated mesh set into the body of the lap;

Fig. XI is a sectional view on the line XI—XI of Fig. X;

Fig. XII is a plan view of a lap having diamond impregnated mesh applied as a surface layer thereon; and

Fig. XIII is a sectional view on the line XIII—XIII of Fig. XII.

In abrading devices such as laps which employ diamond particles as the cutting agent to do the abrading, the diamond particles are held or embedded in a material which gradually wears down as abrading proceeds. For the sake of economy the diamond particles should be firmly held until their useful life ends. If the diamond particles become loosened while their cutting qualities are not yet blunted, or while the particles are still of considerable size, the tool is used up too rapidly for economical operation.

In accordance with our invention, we so embed the diamond particles that as the matrix in which they are embedded gradually wears down they are all held, from first to last, with substantially the same degree of tenacity. This means that a diamond particle of the same size

and sharpness is maintained in operative position for substantially the same length of time, no matter whether this particle is reached towards the beginning or towards the end of the life of the abrading tool as a whole.

In Fig. I, we have conventionally illustrated a diamond lap such as employed for grinding glass to a predetermined spherical surface. The body 10 of the lap is generally of copper or steel which is soft enough to wear down as the diamond particles become used up, but is durable enough to provide a suitable mounting for the particles so long as their useful cutting life lasts.

In accordance with our invention we form a multiplicity of depressions in the body 10, then insert abrasive carrying metal in these depressions and soften the inserted metal by heating, in this way settling the inserted metal into the depressions to form an integral part of the lap.

In the particular embodiment of our invention illustrated in Figs. II, III and IV, we use sheet copper for carrying the diamond particles. Fig. II is a plan view showing the diamond particles which have been caused in any suitable fashion to adhere to the face of the sheet copper 11.

We then fold the diamond carrying sheet of copper 11 about the core 12 of soft iron. This core is selected in suitable dimensions for wedging the sheet 11 in one of a multiplicity of kerfs 14 formed in the lap 10 as diagrammatically illustrated in Fig. IV. It will be noted that the diamond particles are not dislodged from the sheet copper 11 during the inserting step because the particles are firmly held between the copper and the soft iron core.

The kerfs 14 are thus charged with the abrasive carrying metal; and the kerfs are preferably evenly distributed about the body of the lap so as to give a uniform grinding action. The lap is then heat treated under reducing conditions and raised to a temperature sufficiently high to soften or melt the copper. It is desirable to carry on this heat treatment in a reducing atmosphere, but reducing conditions can be obtained in other ways if found more desirable. The whole is then quenched from about 1500° to 1600° F. to give the steel temper. The latter is then drawn to about 25 to 40 on the C. scale, Rockwell, which is the range of hardness generally found suitable for diamond laps.

This treatment hardens the steel sufficiently so that it does not wear down rapidly enough to release the diamond particles before their useful life is finished. The diamond particles are em-

bedded in the copper which under the heat treatment softens enough to flow in around them and forms a matrix of substantially uniform characteristics from top to bottom of the kerf 14.

- 5 The lap may be charged with diamond particles in other ways in accordance with our invention. For example, as illustrated in Fig. V, the diamond particles may be brushed over wire mesh 16, preferably of alloy steel wire which will resist 10 softening at the temperature used for softening the copper. We select the mesh 16 according to the size of the diamond particles, for instance, 100 mesh. When the diamond particles are brushed over the wire mesh, each of the interstices receives a diamond particle so that these particles are quite uniformly distributed.

We find it advantageous to deposit a flash coating of copper over the alloy steel wire before the diamond particles are distributed in the interstices. We then plate the diamond impregnated wire mesh with copper 17, so as to fix the diamond particles in the wire mesh in the manner illustrated in Fig. VI. The abrasive carrying mesh 16 is protected on one or both sides with sheet copper 18, then folded together in a plurality of layers to make up an insert 19, which is pushed into a kerf 14 in the manner indicated in Fig. VII.

The lap is then heat treated under reducing conditions to melt or soften the copper, as set forth in connection with the first embodiment of our invention. Here the wire mesh serves to hold the diamond particles from rising to the surface and thus becoming segregated, while the copper is in softened condition; and therefore the diamond abrasive is uniformly distributed throughout the kerf 14. When the copper hardens again the particles are embedded in a matrix which tenaciously holds the diamond particles as the lap is gradually worn away to expose the underlying particles of abrasive. The lap is quenched and drawn in the manner set forth in connection with the first embodiment of the invention, to control the rate at which the lap wears away.

45 Fig. VIII illustrates a further modification of our invention in accordance with which a mixture of diamond dust and copper or brass particles or chips is forced into each kerf 14. If a brass is used, we prefer to use a brazing brass. 50 After the copper and diamond particles or brass and diamond particles have been carefully mixed, the mixture is forced into the kerfs 14. The lap is then heat treated under reducing conditions to sinter the particles of metal together. In this 55 sintering operation the diamond carrying metal becomes moulded to the contour of the recess 14 in which the metal is received. The body 10 of steel is then quenched and drawn in the manner set forth in connection with the first embodiment of our invention.

60 Control of the heat treating temperature so as not to render the copper or brass liquid, but rather to sinter the metal particles together makes it impossible for the diamond particles to segregate out of the metal during the heat treatment.

A further modification of our invention is illustrated in Figs. IX, X and XI; and here the body 10a of the lap is provided with an annular groove 70 22 for receiving a plurality of layers of diamond impregnated mesh. One of the inserts 23 of diamond impregnated wire mesh is shown in Fig. IX. We prefer to impregnate the wire mesh with the diamond particles and secure the particles in 75 place by the aid of electrolytically deposited cop-

per as described in connection with Figs. V and VI of the drawings. Here the wire mesh is in the shape of an annulus which is of such size as to fit into the groove 22. The successive layers of impregnated wire mesh are separated by sheet 5 copper 24, a sheet of copper being placed on top of a layer of mesh 23, then another layer of mesh, then another sheet of copper and so on until the groove 22 is filled.

The lap is then heat treated under reducing 10 conditions and subsequently quenched and drawn, the practice set forth in connection with Fig. VII being followed.

Instead of inserting the impregnated wire mesh in a depression, groove, or the like, as set forth 15 in connection with Figs. VII, and XI, we may apply the impregnated wire mesh to the surface of the lap which is used in abrading. Figs. XII and XIII illustrate this modification of our invention.

20 The diamond impregnated wire mesh is prepared as set forth in connection with Figs. V, VI and VII. The wire mesh is in the shape of an annulus and is applied to the rounded annular shoulder or rim 26 of the lap as illustrated in 25 Fig. XIII. The edges of the annulus are pressed down so that the wire mesh conforms to the contour of the shoulder and lies snugly against the surface thereof. The lap is then heat treated under reducing conditions to melt or soften the 30 copper as set forth in connection with the preceding embodiments of our invention. As copper diffuses into steel below the softening point of the latter, an excellent bond is thus effected between the diamond impregnated wire mesh and 35 the steel lap. This results in a surface layer of abrasive in which the diamond particles are embedded in copper, the latter being reinforced by steel wire mesh. Inasmuch as the diamond particles are disposed in the interstices of the wire 40 mesh, the diamond particles are each in effect provided with a setting or mounting which affords ample support during the abrading operation until the useful life of the diamond particles is spent.

45 This latter is an important advantage from the point of view of economy. We have discovered that even with a matrix material which is particularly well adapted for retaining the diamond particles during grinding, the particles are inefficiently held if two or more of them are held 50 in a single pocket. In other words, the matrix or embedded material must completely surround each individual particle so that each has its own setting or pocket. The use of the wire mesh into which the diamond particles are brushed is particularly 55 advantageous in insuring that the individual particles are spaced apart and each tenaciously held by its own setting.

The procedure taught herein insures remarkable uniformity in the cutting operation throughout the life of the abrading device, thus promoting economical use of the diamond particles.

60 While we have illustrated and described certain embodiments of our invention, it will be understood that the invention may be otherwise embodied and practiced within the scope of the following claims.

We claim:

1. In a method of producing an abrading device, the steps consisting in forming a slot in the 70 device, dispersing abrasive particles among layers of metal softenable at a lower temperature than said slotted device, inserting said abrasive carrying layers of metal in a slot of said device, and softening the metal with heat after such insertion 75

so as to cause it to conform more nearly to the cross section of said slot.

2. In a method of producing an abrading device, the steps consisting in forming a narrow depression in the device, folding sheet metal to include abrasive particles and form an insert, placing said insert in the depression in said device, and softening the metal with heat after such insertion so as to cause it to conform substantially to the cross-section of said depression.

3. In a method of producing an abrading device, the steps consisting in slotting the device, clamping abrasive particles in folded sheet metal to form an insert, placing said insert in a slot in said device, and softening the metal with heat after such insertion so as to cause it to conform substantially to the cross-section of said slot.

LLOYD W. GODDU.

WILLIAM J. WRIGHTON. 10